

## UNITED STATES PATENT OFFICE

2,091,639

PROCESS FOR THE MELTING, REFINING,  
AND CASTING OF MAGNESIUM AND ITS  
ALLOYSAlfred Claude Jessup, Clamart, France, assignor  
to Societe de Produits Chimiques des Terres  
Rares, Paris, FranceNo Drawing. Application December 2, 1936, Se-  
rial No. 113,938. In Germany December 19,  
1935

5 Claims. (Cl. 75—67)

The casting of magnesium and its alloys gives rise to well known difficulties, owing to the ease with which the molten metal is attacked by air. When the unprotected molten metal is stirred 5 in contact with air, copious formation of oxide and nitride takes place, soon giving rise to inflammation of the entire contents of the crucible, even when the temperature of the metal does not greatly exceed its melting point.

10 It has therefore been constant practice to melt, refine, and cast magnesium and its alloys under a protective covering which prevents attack of the metal by air. This may be done either by the use of inert gases in a completely enclosed 15 crucible, or in the case of open crucibles by means of certain fluxes which form a film between the metal and the atmosphere. It has also been proposed to decrease the inflammability of magnesium and its alloys by incorporating from  $\frac{1}{4}$  to  $\frac{1}{2}\%$  of Ca, in which case the metal can be 20 cast without other protective means. The addition of Ca has in this respect proved beneficial, but the mechanical properties of the metal suffer if the calcium content exceeds 0.05%. This 25 means of protecting the molten metal against attack by the air is therefore only applicable under certain limited conditions.

A very large number of salts and mixtures of salts have heretofore been proposed to enable 30 the metal to be melted, refined and cast out of contact with air. Most of these consist, at least in part, of halogen salts of magnesium, the alkali and the alkaline earth metals. Some of these 35 mixtures having a low melting point are in fact capable of greatly diminishing the attack of the metal during melting, and are also capable of absorbing to a large degree the impurities which it is desired to remove from the metal when it is refined. It has however been found that even 40 when using the best of these fluxes, castings are produced which include a considerable amount of the flux, unless the stirring of the metal is followed by a settling step lasting at least 10 minutes. These foreign particles act in a highly cor- 45 rosive and therefore deleterious manner. The use of such fluxes is therefore impossible in die-casting, where several castings have to be made a minute.

The present invention consists in a process for 50 the melting, refining and casting of magnesium and its alloys, in which attack of the molten metal by air is almost completely obviated, and corrosive inclusions entirely excluded. According to the invention this result is achieved by the 55 use of a flux consisting principally of a substan-

tially eutectic mixture of the fluoride and chloride of calcium or strontium together with barium fluoride.

The efficient action of such a salt mixture is all the more surprising in as much as it is known 5 that a flux consisting of a-eutectic mixture of calcium chloride and calcium fluoride (82%  $\text{CaCl}_2$  18%  $\text{CaF}_2$ ) is inappropriate. It could therefore in no way have been foreseen that satisfactory 10 results could be obtained by simply adding barium fluoride to such a flux, and that in fact such a flux would prove superior to any of the previously known fluxes. Not only do such fluxes containing barium fluoride form a most efficient 15 protective film over the metal against attack by the air, but over and above this they have the great and unexpected advantage that they leave behind no corrosive inclusions even when metal is cast from a pot at the rate of several pours a minute, as is the case in die-casting.

The cause of this fact appears to lie in the 20 high surface tension of the flux in question, which permits the flux spreading out in a thin protective film over the surface of the molten metal, while at the same time preventing it penetrating 25 the surface of the metal and so finding its way into the interior of the melt. For the same reason the film of flux is not inclined to follow the metal when this is poured from the pot. Should however a little flux follow the metal, this always 30 remains on the surface, never in the interior, and can thus be removed by pickling in acid.

The composition of the aforesaid fluxes can 35 vary within somewhat wide limits. On the one hand mixtures on both sides of the eutectic mixture can be employed; and on the other, both calcium chloride and calcium fluoride can be partially or entirely replaced with strontium chloride or fluoride. Too large quantities of barium fluoride should be avoided, as this salt serves 40 rather to reduce the protection the film affords against the air. But within certain limits, the proportions of barium fluoride can also be varied. A few per cent can be employed, but preferably the proportion is maintained somewhat higher. A flux whose composition is particularly well 45 adapted to die-casting has the following composition:

|                 | Per cent |
|-----------------|----------|
| $\text{CaCl}_2$ | 60       |
| $\text{CaF}_2$  | 15       |
| $\text{BaF}_2$  | 25       |

Should it be desired to refine the metal at the same time as it is cast, the molten metal is intimately stirred with the flux, which to a large 55

extent absorbs all impurities present in the metal. The high surface tension of the flux then results in a speedy and complete separation of the flux from the metal.

5 When metal is poured from a large into small crucibles, the surface of the metal in the latter is again protected from attack by the air with a film of the same flux. One can however also dip the metal out of a large pot by means of a ladle, 10 sprinkling a little flux over the metal it contains. Simultaneously, or after adding the flux, one can, in known manner, sprinkle sulphur over the ladle's contents.

The more finely powdered and intimately mixed 15 is the flux, the more efficient is its action.

Having now particularly described and ascertained the nature of my invention and in what manner the same is to be performed, I declare that what I claim is:

20 1. Process for the melting, refining and casting of magnesium and its alloys, which comprises treating the metal with a flux consisting primarily of the chloride of a metal of the group constituted by calcium and strontium and the fluoride

of a metal of the same group, together with barium fluoride.

2. Process according to claim 1, in which the proportions of the chloride and the fluoride of the metals of the group constituted by calcium 5 and strontium, are substantially those existing in one of the eutectic mixtures which the said salts are capable of forming among themselves.

3. Flux for the melting, refining and casting of magnesium and its alloys, consisting of barium 10 fluoride, the chloride of a metal of the group constituted by calcium and strontium and the fluoride of a metal of the same group.

4. Flux according to claim 3, in which the proportions of the chloride and the fluoride of the 15 metals of the group constituted by calcium and strontium, are substantially those existing in one of the eutectic mixtures which the said salts are capable of forming among themselves.

5. Flux according to claim 3, consisting substantially of 25% barium fluoride, 60% calcium chloride and 15% calcium fluoride. 20

ALFRED CLAUDE JESSUP.